

## 1

3,005,759

**ZINC ELECTROPLATING**

William H. Safranek and Hugh R. Miller, Columbus, Ohio, assignors, by mesne assignments, to American Zinc Institute, New York, N.Y., a corporation of New York  
 No Drawing. Filed Apr. 24, 1959, Ser. No. 808,555  
 4 Claims. (Cl. 204—55)

This invention relates to zinc electroplating, and particularly to a method and compositions for electroplating bright, leveling zinc.

One object of the invention is to provide a method for eliminating or reducing the costs of polishing and buffing of die castings prior to electroplating with copper, nickel, and chromium. Heretofore, zinc die castings had to be polished and buffed by costly mechanical procedures to eliminate scratches, pits, cold shut, and other surface irregularities to make their surfaces sufficiently smooth for producing a mirrorlike finish by plating with copper, nickel, and chromium. Although several leveling-type copper and nickel plating processes are employed commercially, they do not result in a satisfactory mirrorlike appearance unless the die cast surfaces are first smoothened mechanically. However, by zinc plating with the process of this invention, a smooth bright finish can be obtained on zinc die castings without the need for polishing or buffing them. When the zinc-plated die castings are subsequently electroplated with leveling copper and nickel, and finally with chromium, an excellent mirrorlike appearance is obtained.

Another object is to provide a method for improving the corrosion resistance of electroplated zinc die castings. It has been established that surface pores in die cast surfaces seldom are removed completely by mechanical polishing or buffing, and it has been established further that such pores, which usually are neither filled nor bridged by copper, nickel, and chromium plating, are the focal points for corrosion when electroplated die castings are exposed outdoors. However, by zinc plating according to this invention, surface pores are filled or bridged with zinc plate. Copper, nickel and chromium then can be electroplated with no discontinuities or pits, thereby improving the corrosion resistance of the electroplated die castings.

A further object of this invention is to provide a method for improving the appearance of zinc-plated steel parts. Although several processes are employed commercially for electroplating bright zinc, they have little or no leveling power and, as a result, steel parts stamped from hot-rolled steel and other parts fabricated from commercial cold-rolled steel with a No. 1 or No. 2 finish have an inferior, frosty or hazy appearance after zinc plating by prior art processes. The appearance of such parts, however, is improved greatly by zinc plating according to the present invention. Surfaces are more nearly mirrorlike and irregularities such as scratches and pits are covered or hidden, because of the exceptional leveling power of the zinc plate deposited by the present process.

Other objects and advantages of the present invention are apparent from the disclosure herein.

It has been found in the present invention that certain critical ranges of composition and operating conditions are necessary to provide optimum polishing of scratches and leveling, especially pore filling.

Table I below lists preferred and useful ranges of bath compositions and operating conditions according to the present invention.

 2  
 TABLE I

|    | Bath constituents                                                                                                                             | Preferred range                                                                                                                                | Useful range                                                                                                            |
|----|-----------------------------------------------------------------------------------------------------------------------------------------------|------------------------------------------------------------------------------------------------------------------------------------------------|-------------------------------------------------------------------------------------------------------------------------|
| 5  | Zinc sulfate, $ZnSO_4 \cdot 7H_2O$ .<br>Ammonium chloride, $NH_4Cl$ .<br>Sodium sulfate, $Na_2SO_4$ .<br>Boric acid, $H_3BO_3$ .              | 1.3 to 1.6 molar.<br>0.15 to 0.4 molar.<br>0.07 to 0.15 molar.<br>0.15 to 0.35 molar.                                                          | 0.8 to 1.8 molar.<br>Optional up to 1.0 molar.<br>0.07 to 0.4 molar.<br>Optional up to 0.7 molar.<br>0.05 to 0.5 molar. |
| 10 | Citrate ions (citric acid and/or sodium citrate).<br>Glycerin.                                                                                | 0.15 to 0.3 molar.<br>0.01 to 0.1 molar.                                                                                                       | Optional up to 0.1 molar.                                                                                               |
| 15 | Saccharin.<br>p-Toluene sulfonamide.<br>Tergitol 08 <sup>1</sup> (wetting agent).<br>pH.                                                      | 0.08 to 0.12 molar.<br>0.005 to 0.02 molar.<br>0.5 to 1.0% by volume.<br>2.3 to 2.5.                                                           | 0.05 to 0.15 molar.<br>0.003 to 0.025 molar.<br>0.3 to 1.5% by volume.<br>2.0 to 3.0.                                   |
| 20 | Operating conditions:<br>Periodic current reversal cycle.<br>Cathode current density (forward and reverse).<br>Temperature.<br>Agitation air. | 14 to 18 seconds direct.<br>8 to 10 seconds reverse.<br>200 to 250 amp./sq. ft.                                                                | 4 to 60 direct.<br>1 to 40 reverse.<br>100 to 350 amp./sq. ft.                                                          |
| 25 | Work bar.<br>Anode current density.<br>Voltage (between anode and cathode).                                                                   | 112 to 120° F.<br>Sufficient to raise solution level $\frac{1}{2}$ to 1 inch.<br>20 to 30 c.p.m.; 2 to 4 inch stroke.<br>30 to 60 amp./sq. ft. | 110 to 130° F.<br>Mild to turbulent.<br>10 to 60 c.p.m.; 1 to 8 inch stroke.<br>10 to 100 amp./sq. ft.                  |
| 30 | Plating time.<br>Plating rate.<br>Thickness of deposit.                                                                                       | 6 to 12 volts.<br>25 to 30 minutes.<br>0.002 to 0.004 inch/hour.<br>0.001 to 0.002 inch.                                                       | 6 to 20 volts.<br>15 to 60 min.<br>0.002 to 0.004 inch/hour.<br>0.0005 to 0.003 inch.                                   |

<sup>1</sup> Tergitol 08 is a 38 percent solution of sodium sulfate derivative of 2-ethyl hexanol-1.



40 The ammonium chloride increases the conductivity of the bath but can be replaced with other highly conducting salts, such as ammonium fluoborate or other ammonium halides. Boric acid and citric acid are buffers. Citric acid and sodium citrate act as aids in promoting leveling power. Glycerin promotes pore filling. Saccharin and p-toluene sulfonamide are the primary brightening agents.

45 The wetting agent prevents pitting. It can be omitted if the bath is maintained in a substantially pure condition, free from oil, common grease, and metallic impurities such as copper, lead, and cadmium.

50 The essentials of the bath composition are (a) zinc sulfate in the range of about 0.8 to 1.8 mols per liter (230 to 500 grams per liter), preferably about 1.3 to 1.6 mols (375 to 450 grams per liter); (b) citrate ions in the range of about 0.05 to 0.5 mol per liter, preferably about 0.15 to 0.3 mol per liter; saccharin in the range of about 0.05 to 0.15 mol per liter (9 to 27 grams per liter), preferably about 0.08 to 0.12 mol per liter (15 to 22 grams per liter); p-toluene sulfonamide in the range of about 0.003 to 0.025 mol per liter (0.5 to 4 grams per liter), preferably about 0.005 to 0.02 mol per liter (0.9 to 3.5 grams per liter); and acid concentration such as to provide a pH in the range of about 2.0 to 3.0, preferably about 2.3 to 2.5.

55 A bath prepared with sodium citrate and no citric acid needs an addition of sulfuric acid to reduce the pH to within the desired range. A bath prepared with citric acid and no citrate salt needs an addition of sodium or ammonium hydroxide to increase the pH to within the desired range. A bath prepared with approximately

equal weights of citric acid and sodium citrate does not require any additional ingredient to adjust the pH.

*Examples*

An extensive study was conducted on the properties of the plates deposited in the following bath:

|                                    |                         |
|------------------------------------|-------------------------|
| Zinc sulfate, $ZnSO_4 \cdot 7H_2O$ | 1.2 mols.               |
| Ammonium chloride, $NH_4Cl$        | 0.08 mol.               |
| Sodium sulfate, $Na_2SO_4$         | 0.05 mol.               |
| Boric acid, $H_3BO_3$              | 0.16 mol.               |
| Citric acid                        | 0.26 mol.               |
| Glycerin                           | 0.08 mol.               |
| Saccharin (soluble sodium salt)    | 0.1 mol.                |
| p-Toluene sulfonamide              | 0.016 mol.              |
| Tergitol 08                        | 0.5 percent, by volume. |

Sodium hydroxide (to raise the pH to about 2.4) Approximately 10 g./l.

This bath was operated for more than two weeks. Operating conditions during this two-week period were in the following ranges:

Temperature 110 to 118 F.  
Current density 150 to 300 amp./sq. ft.

Periodic current reversal cycle:

Direct for 15 seconds  
Reverse for 9 seconds

When the plating conditions were alike, deposits with a consistent bright and leveling appearance were reproduced a number of times. During this period, only a very slight precipitate formed. Judging by the results of holding a few of the crystals in a Bunsen flame, the precipitate was sodium citrate and not saccharin or p-toluene sulfonamide.

Results of other investigations are listed in Table II below.

(glycyrrhizin) gradually coagulated in the plating bath and became inert.

(4) *Improved physical properties.*—Old brightener sometimes was occluded in the zinc deposit; after plating with copper, nickel and chromium and heating the electroplated zinc die castings, blisters sometimes were noted in the electroplated zinc layer as a result of the thermal decomposition of the traces of the occluded glycyrrhizin. Similar heat tests (up to 350° F.) with die castings plated with zinc by the new procedure and then plated with copper, nickel and chromium showed no blistering. Bend tests of zinc-plated steel panels showed a better ductility for the zinc deposited by the new procedure, compared with the zinc deposited by the previous procedure (using glycyrrhizin).

(5) *Simplifies plating bath control.*—The previous bath containing glycyrrhizin had to be continuously filtered to remove coagulated glycyrrhizin; filtration is not required for the new procedure, except for removing dirt accidentally introduced into the plating bath from the air above the solution or from parts being plated. By the old procedure, glycyrrhizin had to be added at frequent intervals to maintain bright, leveling plates. By the new procedure, brighteners are added only at infrequent intervals merely to replace consumption by dragout.

What is claimed is:

1. A method of bright, leveling zinc electroplating comprising plating zinc upon a conductive cathode from a zinc solution consisting essentially of about 1.3 to 1.6 mols per liter of zinc sulfate, about 0.15 to 0.3 mol per liter of citrate ions, about 0.08 to 0.12 mol per liter of saccharin, and about 0.005 to 0.02 mol per liter of p-toluene sulfonamide, said solution having a pH from about 2.3 to 2.5; providing the plating by a periodic current reversal cycle alternating between forward current

TABLE II

EFFECT OF INCREASING THE CATHODE CURRENT DENSITY ON APPEARANCE OF LEVELING ZINC PLATE \*

| Cathode current density, <sup>b</sup><br>amp./sq. ft. | Voltage,<br>volts | Temperature,<br>° F. | Plating<br>time,<br>min. | Rate of<br>deposition,<br>mils/hr. | Appearance of zinc plate                                                        |                                                                     |
|-------------------------------------------------------|-------------------|----------------------|--------------------------|------------------------------------|---------------------------------------------------------------------------------|---------------------------------------------------------------------|
|                                                       |                   |                      |                          |                                    | Before plating with copper, nickel, chromium                                    | After plating with copper, nickel, chromium                         |
| 150                                                   | 3.4               | 117-118              | 50                       | 2.4                                | Very slightly grainy in recesses; nonuniformly semibright.                      | Superior leveling; very slightly hazy at low current density areas. |
| 200                                                   | 4.4               | 116                  | 40                       | 3.2                                | No apparent graininess; uniformly semibright except for slightly dull recesses. | Superior leveling; no graininess; mirror bright.                    |
| 250                                                   | 5.4               | 115-118              | 31                       | 3.85                               | No graininess, uniformly semibright.                                            | Do.                                                                 |
| 300                                                   | 6.4               | 120                  | 25                       | 4.8                                | No graininess, uniformly hazy bright; very slightly burned at top of casting.   | Do.                                                                 |

\* The zinc bath composition was as follows:

|                        |         |               |
|------------------------|---------|---------------|
| $ZnSO_4 \cdot 7H_2O$   | molar   | 1.2           |
| $NH_4Cl$               | do      | 0.08          |
| $H_3BO_3$              | do      | 0.05          |
| Sodium Citrate         | do      | 0.25          |
| $Na_2SO_4$             | do      | 0.05          |
| Glycerin               | do      | 0.08          |
| Saccharin              | do      | 0.1           |
| p-Toluene sulfonamide  | do      | 0.016         |
| Tergitol 08, by volume | percent | 0.5           |
| pH                     |         | $2.4 \pm 0.5$ |

Operating conditions:

PR cycle—

Direct for 15 seconds.

Reverse for 9 seconds.

Agitation: Air plus work bar.

Temperature: 115 to 120° F.

b The current density during the reverse part of the cycle was about 5 percent higher than the current density during the direct part of the cycle.

The present process provides several unexpected advantages over the process of the U.S. Patent 2,905,603 of William H. Safranek and Hugh R. Miller:

(1) *Broader bright plating range.*—Plate is uniformly bright on recesses as well as high current density areas, whereas plate deposited by previous procedure was dull in recesses.

(2) *Better leveling power.*

(3) *Improved brightener stability.*—New brighteners are consumed only by dragout, whereas old brightener

for about 14 to 18 seconds at a cathode current density of about 200 to 250 amperes per square foot and reverse current for about 8 to 10 seconds at a cathode current density of about 200 to 250 amperes per square foot, while maintaining the temperature of said solution between about 112 and 120° F.

2. A composition of matter for bright, leveling zinc electroplating consisting of an aqueous solution consisting essentially of about 1.3 to 1.6 mols per liter of zinc sulfate, about 0.15 to 0.3 mol per liter of citrate ions,

about 0.08 to 0.12 mol per liter of saccharin, and about 0.005 to 0.02 mol per liter of p-toluene sulfonamide, said solution having a pH from about 2.3 to 2.5.

3. A method of bright, leveling zinc electroplating comprising plating zinc upon a conductive cathode from a zinc solution consisting essentially of about 0.8 to 1.8 mols per liter of zinc sulfate, about 0.05 to 0.5 gram per liter of citrate ions, about 0.05 to 0.15 mol per liter of saccharin, and about 0.003 to 0.025 mol per liter of p-toluene sulfonamide, said solution having a pH from about 2.0 to 3.0; providing the plating by a periodic current reversal cycle alternating between forward current for about 4 to 60 seconds at a cathode current density of about 100 to 350 amperes per square foot and reverse current for about 1 to 40 seconds at a cathode current density of about 100 to 350 amperes per square foot, while maintaining the temperature of said solution between about 110 and 130° F.

4. A composition of matter for bright, leveling zinc electroplating consisting of an aqueous solution consist-

10

15

20

ing essentially of about 0.8 to 1.8 mols per liter of zinc sulfate, about 0.05 to 0.5 mol per liter of citrate/ions, about 0.05 to 0.15 mol per liter of saccharin, and about 0.003 to 0.025 mol per liter of p-toluene sulfonamide, said solution having a pH from about 2.0 to 3.0.

#### References Cited in the file of this patent

##### UNITED STATES PATENTS

|           |                 |                |
|-----------|-----------------|----------------|
| 808,103   | Meaker          | Dec. 26, 1905  |
| 2,905,603 | Safranek et al. | Sept. 22, 1959 |

##### FOREIGN PATENTS

|         |               |              |
|---------|---------------|--------------|
| 693,606 | Great Britain | July 1, 1953 |
|---------|---------------|--------------|

##### OTHER REFERENCES

Bray et al.: Transactions, Electrochemical Society, vol. 78 (1940), pp. 309-316.